

# UNITED STATES PATENT OFFICE.

THOMAS B. ALLEN, OF NIAGARA FALLS, NEW YORK, ASSIGNEE TO THE CARBORUNDUM COMPANY, OF NIAGARA FALLS, NEW YORK, A CORPORATION OF PENNSYLVANIA.

## SILICON ARTICLE.

1,073,560.

Specification of Letters Patent. Patented Sept. 16, 1913.

No Drawing.

Application filed January 26, 1912. Serial No. 673,520.

To all whom it may concern:

Be it known that I, THOMAS B. ALLEN, a resident of Niagara Falls, Niagara county, State of New York, have invented a new 5 and useful Improvement in Silicon Articles, of which the following is a full, clear, and exact description.

This invention has relation to a new and useful improvement in silicon articles.

10 Heretofore, the production of silicon articles by casting molten metal into the desired shape has been attended with very great difficulties, which have been so great as to practically prevent the formation of 15 suitable articles. The main difficulties in casting the ordinary molten metal have been, first, that the cast metal is very spongy and porous, being filled with blow holes and pin holes; second, that the cast article is 20 mechanically unsound, this being largely occasioned by the presence of flow marks due to the lapping of the metal which causes folds in the surfaces of the cast silicon; and third, that the cast metal is rather coarsely 25 crystalline.

I have discovered that electric furnace silicon and silicon alloys and compounds contain dissolved silicon dioxid and dissolved nitrogen and oxygen, and that by removing these substances, I am able to obtain castings which are stronger, denser and more perfect than any castings so far obtained. I have further discovered that I can obtain the improvements and remove the 30 impurities by means of a large number of substances, such as the alkali metals, the alkaline earth metals, magnesium, vanadium, titanium, aluminum, boron, etc., and in general, any element which has a combining 35 heat with the impurities, which is greater than that of silicon. To obtain especially advantageous results, I preferably use a material, such as calcium, magnesium, vanadium, etc., which, besides acting as a deoxidizing agent, can act as a denitrogenizing 40 agent. I may, however, also add an element, such as sodium, to remove the oxygen or oxids, and a substance, such as vanadium, to remove the nitrogen or nitrids.

45 I will now describe a preferred method of making an article embodying my invention, with reference to the use of magnesium. I preferably tap the molten silicon from the electric furnace in which it is made into a 50 graphite crucible, and place this crucible in

a coke or oil burning crucible furnace. I then heat the silicon for about one to two hours, having preferably placed a layer of coke on the surface of the silicon to prevent loss by oxidation and volatilization. When 60 the silicon is in a very fluid condition, I remove the crucible from the furnace, skim off the coke and add the magnesium to the molten silicon in the form of a fine powder, or in small lumps, by means of an implement commonly called a "phosphorizer." I have found that I can obtain the desired results by adding from one-half per cent. to three per cent. magnesium, and I contemplate adding only such a quantity of this 65 substance which will combine with the impurities and pass off to the surface of the silicon as a slag. The magnesium silicate formed when magnesium is used is readily fusible and comes to the surface of the fused 70 silicon. When the silicon shows no further reaction due to magnesium and is in a quiescent condition, I preferably pour it from the bottom of the crucible in order to prevent 75 any of the slag from the surface getting into 80 the molten silicon.

In making the mold of the desired shape, for the silicon article, I prefer to use what is commonly known as a dry sand mold and to coat the surfaces of this mold with which 85 the molten silicon comes in contact with talc. I have further found it desirable to pour the metal into the mold through a gate entering at the bottom of the mold and to use a comparatively large "riser," so that 90 the casting cools under considerable fluid pressure. By this means, I aid the production of dense sound castings. The articles produced in this manner are mechanically 95 sound and show a marked absence of blow holes and flow marks. The metal crystallizes in very fine crystals and shows a marked interpenetration of the same which causes articles produced to have considerable mechanical strength.

100 The cast articles are adapted for use for various purposes, being particularly useful as chemical ware on account of their remarkable acid-resisting properties. They are made in the form of pipes, evaporating vessels, receivers, crucibles and pump parts for the concentration and conveyance of acids and acid gases. I do not, however, limit myself to these particular articles.

105 It will be evident to others skilled in the

art of making castings that I may make changes in the described method, without departing from the spirit of the invention. Further, by the term "silicon" used in the following claims, I mean to include the alloys and compounds in which silicon is the principal constituent part.

The novel method herein described forms the subject matter of my Patent No. 10 1,037,713, dated September 3, 1912, for method of making silicon articles.

I claim:

- 15 1. As a new article of manufacture, a cast article having silicon as its principal constituent part and being substantially free from nitrogenous and oxygenous impurities, substantially as described.
- 20 2. As a new article of manufacture, a cast article having silicon as its principal constituent part and being substantially free from nitrogenous and oxygenous impurities, and having a fine crystalline structure, substantially as described.
- 25 3. As a new article of manufacture, a cast article having silicon as its principal con-

stituent part and being substantially free from nitrogenous and oxygenous impurities and being of substantially uniform density throughout its mass, substantially as described. <sup>3</sup>

4. As a new article of manufacture, a cast article having silicon as its principal constituent part, the casting having an even crystalline structure and being substantially free from nitrogenous and oxygenous impurities, and being of substantially uniform density throughout its mass. <sup>3</sup>

5. As a new article of manufacture, a cast article having silicon as its principal constituent part, the casting having a fine <sup>4</sup> crystalline structure and being substantially free from silicon dioxid; substantially as described.

In testimony whereof, I have hereunto set my hand.

THOS. B. ALLEN.

Witnesses:

T. B. HUMPHRIES,  
GEO. H. PARMELEE.